

# UNITED STATES PATENT OFFICE.

ALEXANDER JUST AND FRANZ HANAMAN, OF BUDAPEST, AUSTRIA-HUNGARY, AS-SIGNORS, BY DIRECT AND MESNE ASSIGNMENTS, TO GENERAL ELECTRIC COMPANY, A CORPORATION OF NEW YORK.

## INCANDESCENT BODIES FOR ELECTRIC LAMPS.

1,018,502.

Specification of Letters Patent.

Patented Feb. 27, 1912.

No Drawing.

Application filed July 6, 1905. Serial No. 268,523.

*To all whom it may concern:*

Be it known that we, ALEXANDER JUST, chemist, and FRANZ HANAMAN, chemical engineer, subjects of the Emperor of Austria-Hungary, residing at Desewffy utcza 3, Budapest, in the Empire of Austria-Hungary, have jointly invented certain new and useful Incandescent Bodies for Electric Lamps, of which the following is a specification.

10 The present invention has for its object incandescent filaments for incandescent electric lights or lamps which are composed of substantially pure tungsten.

15 Incandescent filaments of this kind may be manufactured in accordance with processes hereinafter described.

One such process is started with bodies consisting of a mixture of tungsten and organic binding media. Such bodies are carbonized and thereupon the carbon is removed by chemical means, the remaining filament or body consisting therefore purely of tungsten. Instead of using tungsten in the first step of manufacture we may also 25 employ compounds of tungsten.

In order to produce filaments consisting of a mixture of tungsten and carbon, finely divided tungsten, or some tungsten compound which is readily reduced by carbon 30 to a metal, such as tungsten oxid, tungstic acid, tungsten sulfid or the like is mixed with an organic binding medium, such as solution of cellulose in chlorid of zinc, collodion, coal tar, coal pitch or the like, the 35 filaments being then formed by pressure in the usual manner and thereupon (or after a preceding denitration in case of applying collodion) these filaments are carbonized. As regards the quantity of the 40 tungsten compound employed in this mixture the proportions should be determined in such a manner that in the finished filaments sufficient carbon is present to impart the requisite strength to them as it is the 45 carbon alone that imparts to such a filament the necessary strength for withstanding the subsequent treatment. Thus for example, efficient filaments are obtained, if from 2 to 10 g. tungstic acid are added to a 50 solution of 10 g. cellulose in 260 g. chlorid of zinc of the specific weight of 1.83, this mixture being then formed into filaments and carbonized in absence of air. The said

filaments which consist of a homogeneous mixture of carbon and tungsten and which are to be regarded as intermediate products, in accordance with the present process are treated in such a way that the carbon is removed therefrom by chemical means. This may be effected, for example, by submitting 55 the filament to the action of an electric current and raising it to a high temperature in an atmosphere of steam and hydrogen. In this process the carbon, analogously to the water-gas process, is completely oxidized 60 into carbonic oxid, and there remains a filament of tungsten. These filaments then may be equalized in a manner analogous to that employed in the treatment of ordinary carbon filaments, by submitting them to the 65 action of a current in an atmosphere of volatile tungsten compounds in the presence of a considerable quantity of hydrogen, so that the tungsten deposited equalizes the filaments. The filaments so produced are fused 70 in the customary manner into glass bulbs, which are then exhausted. Finally tungsten 75 incandescent filaments may be manufactured in the following manner:—As is already known, it is old to coat carbon filaments with 80 tungsten by heating such filaments in the vapor of a halogen compound of this metal in the presence of a large quantity of hydrogen. The finest possible carbon filaments (of about 0.04 mm. in diameter) are coated 85 with a layer of sufficient thickness of the said metal and the filaments are then treated in the following manner: The filaments are exposed in an atmosphere of neutral gases under the influence of an electric current to 90 a high temperature, whereby in a few minutes the carbon contained in the core is dissolved by the metal surrounding it. This solution takes place owing to the fact that the free carbon is absorbed by the metal as 95 carbid. A filament treated in this manner shows itself to be perfectly homogeneous, if a point of fracture is submitted to microscopic inspection, which affords proof that it no longer contains any carbon core. 100 These filaments may now be readily freed from carbon as described above so that pure metal filaments are obtained.

The filaments produced according to this invention consist of dense coherent tungsten 105 metal and have a high fusing point of ap-

proximately 3200° C. and are capable of incandescent efficiency at the rate of less than 1 watt per candle power and are substantially free from perceptible disintegration at that efficiency, the light-emitting properties of the filaments being due to the coherent, homogeneous metallic nature of the tungsten.

What we claim herein as new and desire to secure by Letters Patent is:—

- 5 1. A filament for incandescent lights consisting of tungsten in a coherent metallic state and homogeneous throughout.
- 10 2. A filament for incandescent lights consisting throughout of substantially pure metallic tungsten of high fusing point and electrically conductive, the light emitting properties of the filament being due to the

coherent, homogeneous metallic nature of the tungsten.

3. A filament for electric incandescent lights comprising dense, coherent tungsten metal, having its fusing point approximately 20 3200° C. and capable of incandescent efficiency at the rate of less than 1 watt per candle power and substantially free from perceptible disintegration at that efficiency. 25

In testimony whereof we have signed our names to this specification in the presence of two subscribing witnesses.

ALEXANDER JUST.  
FRANZ HANAMAN.

Witnesses:

LUDVIG ITABORY,  
LOUIS VANDORY.